

## UNITED STATES PATENT OFFICE.

HARRY P. BASSETT, OF CYNTHIANA, KENTUCKY, AND SAMUEL S. SADTLER, OF SPRINGFIELD TOWNSHIP, MONTGOMERY COUNTY, PENNSYLVANIA.

## METHOD OF OBTAINING ARSENIOUS OXIDE.

No Drawing.

Application filed February 25, 1924. Serial No. 695,100.

*To all whom it may concern:*

Be it known that we, HARRY P. BASSETT and SAMUEL S. SADTLER, citizens of the United States, residing at Cynthiana, in the 5 county of Harrison and State of Kentucky, and Springfield Township, in the county of Montgomery and State of Pennsylvania, respectively, have invented certain new and useful Improvements in Methods of Obtaining Arsenious Oxide, of which the following is a specification.

Our invention relates to an economical method of obtaining arsenious oxide from naturally occurring ores of arsenic, such as 15 speisses, mispickels, realgar, orpiment, in which arsenic exists essentially as sulphide or compound sulphide with other metals containing arsenic.

An important object of the invention is 20 the provision of methods of treating such ores which are more economical than any now practiced in the production or recovery of arsenic as a valuable product or by-product. Our process of separating arsenic as it occurs as speisses, mispickels, and in association with sulphur and heavy metals broadly, 25 consists in controlled heating of finely powdered ore at relatively low temperatures and with slight and regulated admission of air. Under such circumstances the arsenic 30 is evolved and leaves the sulphur combined with iron, nickel, cobalt, or other heavy metals, or metals with which the arsenic occurs.

35 We are aware of attempts to remove arsenic as disclosed by Ernest W. Westcott, in United States Patent No. 1,406,597, granted February 14, 1922, in which chlorine is used to combine with the arsenic and render it volatile. This is, however, 40 distinctly different from the present invention. The British patent to Oxland and Hockings, No. 2,950, of 1868, relates to revolving calciners and refers to the fact that 45 arsenic comes off first but it shows no means for controlling the heat and air admission. They completely oxidize the ore. This is in fact what has been and is now the practice at smelters. They drive off both arsenic and 50 sulphur. Oxland and Hockings, furthermore, did not recognize one of the features of our invention, as applied especially to speisses, etc., that is necessary for low temperature and high yield results: namely, the 55 presence of at least combining equivalents

(with reference to the sulphur) of metals forming stable sulphides at temperatures prevailing in this low temperature heating and distillation.

In practicing the invention, we use muffle 60 furnaces, preferably rotary, taking the necessary precautions to avoid a flame that is too strongly oxidizing. The temperatures we have found necessary are so low, however, that we prefer to use the former 65 method, namely, muffle heating.

In a typical embodiment of the invention, the ore is finely ground, say to 100 mesh, and there may be added coke or some other form of carbon or even a little carbon alone, to 70 prevent any burning of the ore. The addition of carbon, however, should not be found necessary with sulphides, if the heat is carefully controlled. In our preferred form of apparatus, we use a substantially closed iron 75 tube without fire brick, which is slowly revolved at a suitable inclination in a flue from a relatively small fire box. The powdered ore or ore mixture passes down through the tube to an ore trap at the lower end. The 80 arsenic fumes with varying amounts of arsenious oxide (depending upon the admission of air) pass upwards to oxidizing and condensing chambers and filters. The temperature in the tube is usually distinctly below 85 red heat. We have used temperatures between 200° C. and 400° C., but especially avoid any temperatures as high as even dull redness unless there is sufficient carbon to protect the ore, when higher temperatures may be used. 90 The arsenic is recovered as arsenious oxide (white arsenic). Enough air may be admitted into the furnace to just burn the arsenic evolved from the ore, but we prefer to admit air above the ore and near the flue 95 entrance so that it does not actually come in contact with the ore except in an attenuated state.

An alternative to this procedure is to admit no air to the muffle and to oxidize the 100 evolved arsenic in the receiving chamber, but we prefer to oxidize the arsenic in the upper part of the muffle. If a small amount of carbon is admixed with the ore, there is less danger of burning the ores. 105

The main reaction involved seems to be:



While we have described in detail the preferred practice of our process, it is to be 110

understood that the details of procedure, and proportion of ingredients may be widely varied, and that known chemical equivalents may be employed in place of the materials mentioned, without departing from the spirit of the invention or the scope of the subjoined claims.

We claim:

1. The method of obtaining arsenious oxide from ores containing arsenic associated with sulfur and heavy metals which comprises heating the ore to a regulated temperature in the presence of a limited amount of air insufficient to oxidize the sulfur present.
2. The method of obtaining arsenious oxide from ores containing arsenic associated with sulfur and heavy metals, which comprises heating the ore to a temperature below 400° C. in the presence of sufficient amount of air to oxidize the evolved arsenic.
3. The method of obtaining arsenious oxide from ores containing arsenic associated with sulfur and heavy metals which comprises heating the ore to a temperature

between 200° C. and 400° C. in the presence of sufficient air to oxidize the evolved arsenic.

4. The method of obtaining arsenious oxide from ores containing arsenic associated with sulfur and heavy metals which comprises reducing the ore to a powder, adding carbon thereto, and heating to a temperature below 400° C. in the presence of a limited amount of air insufficient to oxidize the sulfur present.

5. The process of obtaining arsenious oxide from ores consisting of sulphides of arsenic and other metals which comprises heating the ore at a low temperature such as will release the arsenic and form sulphides of the other metals, and admitting sufficient air to oxidize the evolved arsenic to the tri-oxide.

In testimony whereof, we affix our signatures in presence of a witness.

HARRY P. BASSETT.  
SAMUEL S. SADTLER.

Witness:

A. M. STOKES.